

# United States Patent

[11] 3,607,257

[72] Inventor **Arthur L. Johnson**  
**Rochester, N.Y.**  
[21] Appl. No. **755,711**  
[22] Filed **Aug. 27, 1968**  
[45] Patented **Sept. 21, 1971**  
[73] Assignee **Eastman Kodak Company**  
**Rochester, N.Y.**

[54] **PHOTOCOCONDUCTIVE COMPOSITIONS AND ELEMENTS**  
**33 Claims, No Drawings**

[52] U.S. Cl..... **96/1.6,**  
**96/1.5, 96/1 PC, 260/429 R, 260/448 A, 252/501**  
[51] Int. Cl..... **G03g 5/04**  
[50] Field of Search..... **96/1.5-1.7;**  
**260/429, 448, 45.75; 252/501**

[56]

## References Cited

### UNITED STATES PATENTS

|           |         |                       |           |
|-----------|---------|-----------------------|-----------|
| 2,800,559 | 7/1957  | Ubbelohde .....       | 96/1.5 X  |
| 3,016,397 | 1/1962  | Walde .....           | 260/429 X |
| 3,114,633 | 12/1963 | Schlesinger .....     | 96/1.6    |
| 3,141,770 | 7/1964  | Davis et al. .....    | 96/1.5    |
| 3,163,532 | 12/1964 | Schlesinger .....     | 96/1.5    |
| 3,193,566 | 7/1965  | Wicklitz et al. ..... | 260/429 X |
| 3,409,655 | 11/1968 | Seki et al. .....     | 260/448   |

Primary Examiner—Charles E. Van Horn

Attorneys—William H. J. Kline, James R. Frederick and Fred L. Denson

**ABSTRACT:** Photoconductive compositions and elements containing as photoconductors organometallic compounds derived from Group IIIa metals are described.

## PHOTOCONDUCTIVE COMPOSITIONS AND ELEMENTS

This invention relates to electrophotography and in particular to photoconductive compositions and elements.

The process of xerography, as disclosed by Carlson in U.S. Pat. No. 2,297,691, employs an electrophotographic element comprising a support material bearing a coating of a normally insulating material whose electrical resistance varies with the amount of incident electromagnetic radiation it receives during an imagewise exposure. The element, commonly termed a photoconductive element, is first given a uniform surface charge, generally in the dark after a suitable period of dark adaptation. It is then exposed to a pattern of actinic radiation which has the effect of differentially reducing the potential of this surface charge in accordance with the relative energy contained in various parts of the radiation pattern. The differential surface charge or electrostatic latent image remaining on the electrophotographic element is then made visible by contacting the surface with a suitable electroscopic marking material. Such marking material or toner, whether contained in an insulating liquid or on a dry carrier, can be deposited on the exposed surface in accordance with either the charge pattern or in the absence of charge pattern as desired. Deposited marking material can then be either permanently fixed to the surface of the sensitive element by known means such as heat, pressure, solvent vapor, or the like, or transferred to a second element to which it can similarly be fixed. Likewise, the electrostatic latent image can be transferred to a second element and developed there.

Various photoconductive insulating materials have been employed in the manufacture of electrophotographic elements. For example, vapors of selenium and vapors of selenium alloys deposited on a suitable support and particles of photoconductive zinc oxide held in a resinous, film-forming binder have found wide application in the present day document-copying applications.

Since the introduction of electrophotography, a great many organic compounds have also been screened for their photoconductive properties. As a result, a very large number of organic compounds have been known to possess some degree of photoconductivity. Many organic compounds have revealed a useful level of photoconduction and have been incorporated into photoconductive compositions.

Typical of these organic photoconductors are the triphenylamines and the triarylmethane leuco bases. Optically clear photoconductor-containing elements having desirable electrophotographic properties can be especially useful in electrophotography. Such electrophotographic elements can be exposed through a transparent base if desired, thereby providing unusual flexibility in equipment design. Such compositions, when coated as a film or layer on a suitable support, also yield an element which is reusable; that is, it can be used to form subsequent images after residual toner from prior images has been removed by transfer and/or cleaning. Thus far, the selection of various compounds for incorporation into photoconductive compositions to form electrophotographic layers has proceeded on a compound-by-compound basis. Nothing as yet has been discovered from the large number of different photoconductive substances tested which permits effective prediction, and therefore selection of the particular compounds exhibiting the desired electrophotographic properties.

It is, therefore, an object of this invention to provide a novel class of photoconductors having high photosensitivity when electrically charged.

It is another object to provide novel photoconductor-containing compositions which exhibit high electrical speeds.

It is also an object to provide novel photoconductor-containing compositions which can be positively and negatively charged.

It is another object to provide novel transparent electrophotographic elements having high-speed characteristics.

It is a further object of this invention to provide novel electrophotographic elements useful for producing images electrophotographically by reflex or bireflex processes.

These and other objects of this invention are accomplished with electrophotographic elements having coated thereon photoconductive compositions containing as photoconductors organometallic compounds having at least one amino-aryl substituent attached to a Group IIIa metal atom.

The metallic substituents of these organometallic photoconductors are Group IIIa metals in accordance with the Periodic Table of the Elements (Handbook of Chemistry and Physics, 38th edition, pp. 394-95) and include boron, aluminum, gallium, indium and thallium. The organometallic photoconductors of this invention can be substituted in the metallo nucleus with a wide variety of substituents but at least one of the substituents should be an amino-aryl radical. The amino radical can be positioned anywhere on the aromatic nucleus, but best results are obtained if the aryl moiety is a phenyl radical having the amino group in the 4 or para position. Typical substituents attached to the metal nucleus include the following:

- a hydrogen atom;
- an alkyl group including substituted alkyl groups such as an aralkyl group e.g., benzyl, a halo-alkyl group e.g., a chloromethylene group, and aminoalkyl group e.g.,  $-\text{CH}_2-\text{N}(\text{Et})_2$ , etc.;
- an aryl group such as phenyl, naphthyl, etc.; including substituted aryl groups such as aminoaryl e.g.,



wherein  $\text{R}_1$ ,  $\text{R}_2$  are each a hydrogen atom, an alkyl group including a substituted alkyl group such as an aralkyl group or an aryl group including a substituted aryl group such as an alkaryl group or a haloaryl group;

- an oxygen-containing group such as an alkoxy or aryloxy group;
- an amino group e.g.,  $-\text{NH}_2$  including substituted amino groups such as dialkylamino, diphenylamino, alkylamino, phenylamino, etc.; and
- a Group IIIa organometallic group e.g.,



$\text{M}$  being a Group IIIa metal and  $\text{R}_9$  and  $\text{R}_{10}$  being any of the substituents set forth in a. through e. above.

Illustrative photoconductors of this invention preferably have the following structure:



wherein:

- $\text{D}$  and  $\text{E}$  can be either
- a hydrogen atom;
- an aryl group including substituted and unsubstituted aryl groups such as phenyl, naphthyl, dialkylaminophenyl, dialkylaminonaphthyl, etc.;
- an alkyl group having 1 to 8 carbon atoms;
- an alkoxy group having 1 to 8 carbon atoms;
- an aryloxy group such as a phenoxy group or;
- an amino group e.g.,



$\text{R}_3$  and  $\text{R}_4$  each being a hydrogen atom, an alkyl group or an aryl group;

Ar is an arylene group including a substituted arylene group e.g., a phenylene group, a naphthylene group, an alkylphenylene group, a halophenylene group, etc.;

M is a Group IIIa metal;

R<sub>1</sub> and R<sub>2</sub> can be either

- a. a hydrogen atom,
- b. an alkyl group having 1 to 8 carbon atoms or
- c. an aryl group such as a phenyl or naphthyl group

Particularly improved results are obtained when those photoconductors having the following structure are used:



wherein:

M, D, E, R<sub>1</sub> and R<sub>2</sub> are the same as defined above and T, X and Z can be either

- a. a hydrogen atom,
- b. an alkyl group having 1 to 8 carbon atoms,
- c. an aryl group including a substituted aryl group 20 e.g., phenyl, naphthyl, tolyl halophenyl, aminophenyl, etc.,
- d. an alkoxy group having 1 to 8 carbon atoms,
- e. an aryloxy group such as a phenoxy group,
- f. a halogen atom such as chlorine, bromine or iodine or,
- g. an amino group e.g.,



R<sub>7</sub> and R<sub>8</sub> each being a hydrogen atom, an alkyl group having 1 to 8 carbon atoms or an aryl group such as phenyl or naphthyl. X, T and Z can be the same or different and can be positioned in the 2, 3, 5 or 6 positions on the phenylene ring.

Some typical organometallic photoconductors of this invention include:

TABLE I

1. Tri-p-diethylaminophenylborane
2. Tri-p-diphenylaminophenylborane
3. Tri-p-methylaminophenylgallium
4. Methyl-phenyl-p-diethylaminophenylborane
5. 2 Naphthyl-p-dimethylaminophenylborane
6. p-Dipropylaminophenylborane
7. Di-p-diethylaminophenylborane
8. Ethoxy-p-dimethylaminophenyl aluminum hydride
9. Diphenoxy-p-dibutylaminophenyl aluminum
10. Tri-(2,2-dimethyl-4-diethylaminophenyl)indium
11. 2-chloro-4-dimethylaminophenyl gallium hydride
12. Tri-(2,6-diphenoxy-4-diethylaminophenyl)thallium
13. Tri-(2,6-dimethoxy-4-diethylaminophenyl)thallium
14. Diphenylamino-p-diethylaminophenylborane
15. Dimesityl-4-dimethylaminonaphthylborane
16. Dimesityl-4-dimethylaminophenylborane
17. Dimesityl-(3,5-dimethyl-4-methoxyphenyl)borane
18. Dimesityl-4-diphenylaminophenylborane
19. 1,2Bis(p-diethylaminophenyl)diborane
20. 1-Phenyl-2-methyldiborane

Electrophotographic elements of the invention can be prepared with the photoconducting compounds of the invention in the usual manner, i.e., by blending a dispersion or solution or a photoconductive compound together with a binder, when necessary or desirable, and coating or forming a self-supporting layer with the photoconductor-containing material. Mixtures of the photoconductors described herein can be employed. Likewise, other photoconductors known in the art can be combined with the present photoconductors. In addition, supplemental materials useful for changing the spectral

sensitivity or electrophotosensitivity of the element can be added to the composition of the element when it is desirable to produce the characteristic effect of such materials.

Sensitizing compounds useful with the photoconductive

- 5 compounds of the present invention can include a wide variety of substances such as pyrylium salts including thiapyrylium and selenapyrylium salts of U.S. Pat. No. 3,250,615, issued May 10, 1966; fluorenes, such as 7,12-dioxo-13-dibenzo(a,h)fluorene, 5,10-dioxo-4a,11
- 10 diazabenzoc(b)fluorene, 3,13-dioxo-7-ox-adibeno(b,g)fluorene, trinitrofluorenone, tetranitrofluorenone and the like; aromatic nitro compounds of U.S. Pat. No. 2,610,120; anthrones of U.S. Pat. No. 2,670,285; quinones of U.S. Pat. No. 2,670,286; benzophenones of U.S. Pat. No. 2,670,287; thiazoles of U.S. Pat. No. 2,732,301; mineral acids; carboxylic acids, such as maleic acid, dichloroacetic acid, and salicylic acid; sulfonic and phosphoric acids; and various dyes such as triphenylmethane, diarylmethane, thiazine, azine, oxazine, xanthene, phthalein, acridine, azo, anthraquinone dyes and many other suitable sensitizing dyes. The preferred sensitizers for use with the compounds of this invention are pyrylium salts including selenapyrylium and thiapyrylium salts, fluorenes, carboxylic acids, and triphenylmethane dyes.

Where a sensitizing compound is to be used within a photoconductive layer as disclosed herein it is conventional practice to mix a suitable amount of the sensitizing compounds with the coating composition so that, after thorough mixing the sensitizing compound is uniformly distributed throughout the desired layer of the coated element. In preparing the photoconducting layers, no sensitizing compound is needed for the layer to exhibit photoconductivity. The lower limit of sensitizer required in a particular photoconductive layer is, therefore, zero. However, since relatively minor amounts of sensitizing compound give substantial improvement in the electrophotographic speed of such layers, the use of some sensitizer is preferred. The amount of sensitizer that can be added to a photoconductor incorporating layer to give effective increases in speed can vary widely. The optimum concentration in any given case will vary with the specific photoconductor and sensitizing compound used. In general, substantial speed gains can be obtained where an appropriate sensitizer is added in a concentration range from about 0.0001 to about 30 percent by weight based on the weight of the film-forming coating composition. Normally, a sensitizer is added to the coating composition in an amount by weight from about 0.005 to about 5.0 percent by weight of the total coating composition.

- 45 50 Preferred binders for use in preparing the present photoconductive layers are film-forming, hydrophobic polymeric binders having fairly high dielectric strength which are good electrically insulating film-forming vehicles. Materials of this type comprise styrene-butadiene copolymers; silicone resins; styrene-alkyd resins; silicone-alkyd resins; soy-alkyd resins; poly (vinyl chloride); poly(vinylidene chloride); vinylidene chloride-acrylonitrile copolymers; poly(vinyl acetate); vinyl acetate-vinyl chloride copolymers; poly(vinyl acetals), such as poly(vinyl butyral); polyacrylic and methacrylic esters, such as poly(methylmethacrylate), poly(n-butylmethacrylate), poly(isobutyl methacrylate), etc.; polystyrene; nitrated polystyrene; polymethylstyrene; isobutylene polymers; polyesters, such as poly (ethylenealkylolxyalkylene terephthalate); phenoformaldehyde resins; ketone resins; polyamides; polycarbonates; polythiocarbonates; poly(ethyleneglycol-co-bishydroxyethoxyphenol propane terephthalate); copolymers of vinyl haloarylates and vinyl acetate such as poly(vinyl-m-bromobenzoate-covinylacetate); etc. Methods of making resins of this type have been described in the prior art, for example, styrene-alkyd resins can be prepared according to the method described in U.S. Pat. Nos. 2,361,019 and 2,258,423. Suitable resins of the type contemplated for use in the photoconductive layers of the invention are sold under such tradenames as Vitel PE-101, Cymac, Pic-

copale 100, Saran F-220, Lexan 105 and Lexan 145. Other types of binders which can be used in the photoconductive layers of the invention include such materials as paraffin, mineral waxes, etc.

Solvents of choice for preparing coating compositions of the present invention can include a number of solvents such as benzene, toluene, acetone, 2-butanone, chlorinated hydrocarbons, e.g., methylene chloride, ethylene chloride, etc., ethers e.g., tetrahydrofuran, or mixtures of these solvents, etc.

In preparing the coating composition useful results are obtained where the photoconductor substance is present in an amount equal to at least about 1 weight percent of the coating composition. The upper limit in the amount of photoconductor substance present can be widely varied in accordance with usual practice. In those cases where a binder is employed, it is normally required that the photoconductor substance be present in an amount from about 1 weight percent of the coating composition to about 99 weight percent of the coating composition. A preferred weight range for the photoconductor substance in the coating composition is from about 10 weight percent to about 60 weight percent.

Coating thicknesses of the photoconductive composition on a support can vary widely. Normally, a coating in the range of about 0.001 inch to about 0.01 inch before drying is useful for the practice of this invention. The preferred range of coating thickness was found to be in the range from about 0.002 inch to about 0.006 inch before drying although useful results can be obtained outside of this range.

Suitable supporting materials for coating the photoconductive layers of the present invention can include any of a wide variety of electrically conducting supports, for example, paper (at a relative humidity above 20 percent); aluminum-paper laminates; metal foil such as aluminum foil, zinc foil, etc.; metal plates, such as aluminum, copper, zinc, brass, and galvanized plates; vapor deposited metal layers such as silver or aluminum and the like. An especially useful conducting support can be prepared by coating a support material such as polyethylene terephthalate with a layer containing a semiconductor dispersed in a resin. Such conducting layers both with and without insulating barrier layers are described in U.S. Pat. No. 3,245,833. Likewise, a suitable conducting coating can be prepared from the sodium salt of a carboxyester lactone maleic anhydride and a vinyl acetate polymer. Such kinds of conducting layers and methods for their optimum preparation and use are disclosed in U.S. Pat. Nos. 3,007,901 and 3,267,807.

The elements of the present invention can be employed in any of the well-known electrophotographic processes which require photoconductive layers. One such process is the aforementioned xerographic process. As previously explained, in a process of this type the electrophotographic element is given a blanket electrostatic charge by placing the same under a corona discharge which serves to give a uniform charge to the surface of the photoconductive layer. This charge is retained by the layer owing to the substantial insulating property of the layer, i.e., the low conductivity of the layer in the dark. The electrostatic charge formed on the surface of the photoconducting layer is then selectively dissipated from the surface of the layer by exposure to light through an image-bearing transparency by a conventional exposure operation such as, for example, by contact printing technique, or by lens projection of an image, etc., to form a latent image in the photoconducting layer. By exposure of the surface in this manner, a charged pattern is created by virtue of the fact that light causes the charge to be conducted away in proportion to the intensity of the illumination in a particular area. The charge pattern remaining after exposure is then developed, i.e., rendered visible, by treatment with a medium comprising electrostatically attractive particles having optical density. The developing electrostatically attractive particles can be in the form of a dust, e.g., powder, pigment in a resinous carrier, i.e., toner, or a liquid developer may be used in which the developing particles are carried in an electrically insulating liquid carrier. Methods of development of this type are widely known and

have been described in the patent literature in such patents, for example, as U.S. Pat. No. 2,297,691 and in Australian Pat. 212,315. In processes of electrophotographic reproduction such as in xerography, by selecting a developing particle

which has as one of its components, a low-melting resin, it is possible to treat the developed photoconductive material with heat and cause the powder to adhere permanently to the surface of the photoconductive layer. In other cases, a transfer of the image formed on the photoconductive layer can be made to a second support, which would then become the final print. Techniques of the type indicated are well known in the art and have been described in a number of U.S. and foreign patents, such as U.S. Pats. Nos. 2,297,691 and 2,551,582, and in "RCA Review," vol. 15 (1954), pages 469-484.

The present invention is not limited to any particular mode of use of the new electrophotographic materials, and the exposure technique, the charging method, the transfer (if any), the developing method, and the fixing method as well as the materials used in these methods can be selected and adapted to the requirements of any particular technique.

Electrophotographic materials according to the present invention can be applied to reproduction techniques wherein different kinds of radiations, i.e., electromagnetic radiations as well as nuclear radiations, can be used. For this reason, it is pointed out herein that although materials according to the invention are mainly intended for use in connection with methods comprising an exposure, the term "electrophotography" wherever appearing in the description and the claims, is to be interpreted broadly and understood to comprise both xerography and xeroradiography.

The invention is further illustrated by the following examples which include preferred embodiments thereof.

#### EXAMPLE I

Tri-p-diethylaminophenylborane is separately incorporated into a coating dope have the following composition:

- a. 0.25 gram of Lexan 145 (trade name of General Electric Company for poly(4,4'-isopropylidenediphenylcarbonate as a binder
- b. 0.25 gram of tri-p-diethylaminophenylborane as a photoconductor
- c. 4.5 grams of a 0.0029 g./ml. solution of [4-(p-dimethylaminophenyl)-2,6-diphenylthiapyrylium perchlorate] in methylene chloride as a sensitizer for the photoconductor
- d. 7.7 grams of a composition \*

\*Prepared by the method described in U.S. Ser. No. 674,005 filed Oct. 9, 1967 by W. A. Light containing 3.92 grams of Lexan 145, 0.008 g. of [4-(p-dimethylaminophenyl)-2,6-diphenylthiapyrylium perchlorate] and 26.8 ml. of methylene chloride. The resulting composition is handcoated at a wet thickness of 0.006 inch on a conducting layer comprising the sodium salt of a carboxyester lactone, such as described in U.S. Pat. No. 3,120,028, which in turn is coated on a cellulose acetate film base. The coating blocks are maintained at a temperature of 90° F. These electrophotographic elements are charged under positive or negative corona source until the surface potentials, as measured by an electrometer probe, reach about 600 volts. They are then subjected to exposure from behind a stepped density gray scale to a 3000° K. tungsten source. The exposure causes reduction of the surface potentials of the elements under each step of the gray scale from their initial potential,  $V_0$ , to some lower potential,  $V$  whose exact value depends on the actual amount of exposure in meter-candle-seconds received by the areas. The results of the measurements are plotted on a graph of surface potential  $V$  vs. log exposure for each step. The shoulder speed is the numerical expression of  $10^4$  multiplied by the reciprocal of the exposure in meter-candle-seconds required to reduce the 600-volt-charged surface potential by 100 volts. The toe speed is the numerical expression of  $10^4$  multiplied by the reciprocal of the exposure in meter-candle-seconds required to reduce the 600-volt-charged surface potential to 100 volts. The above composition has positive and negative shoulder speeds of 2,500 and 3,400 respectively. Positive and negative toe speeds are 250 and 900 respectively.

60

65

70

75

500

550

600

650

700

750

800

850

900

950

1000

1050

1100

1150

1200

1250

1300

1350

1400

1450

1500

1550

1600

1650

1700

1750

1800

1850

1900

1950

2000

2050

2100

2150

2200

2250

2300

2350

2400

2450

2500

2550

2600

2650

2700

2750

2800

2850

2900

2950

3000

3050

3100

3150

3200

3250

3300

3350

3400

3450

3500

3550

3600

3650

3700

3750

3800

3850

3900

3950

4000

4050

4100

4150

4200

4250

4300

4350

4400

4450

4500

4550

4600

4650

4700

4750

4800

4850

4900

4950

5000

5050

5100

5150

5200

5250

5300

5350

5400

5450

5500

5550

5600

5650

5700

5750

5800

5850

5900

5950

6000

6050

6100

6150

6200

6250

6300

6350

6400

6450

6500

6550

6600

6650

6700

6750

6800

6850

6900

6950

7000

7050

7100

7150

7200

7250

7300

7350

7400

7450

7500

7550

7600

7650

7700

7750

7800

7850

7900

7950

8000

8050

8100

8150

8200

8250

8300

8350

8400

8450

8500

8550

8600

8650

8700

8750

8800

8850

8900

8950

9000

9050

9100

9150

9200

9250

9300

9350

9400

9450

9500

9550

9600

9650

9700

9750

9800

9850

9900

9950

10000

10050

10100

10150

10200

10250

10300

10350

10400

10450

10500

10550

10600

10650

10700

10750

10800

10850

10900

10950

11000

11050

11100

11150

11200

11250

11300

11350

11400

11450

11500

11550

11600

11650

11700

11750

11800

11850

11900

11950

12000

12050

12100

12150

12200

12250

12300

12350

12400

12450

12500

12550

12600

12650

12700

12750

12800

12850

12900

12950

13000

13050

13100

13150

13200

13250

13300

13350

13400

13450

13500

13550

13600

13650

13700

13750

13800

13850

13900

13950

14000

14050

14100

14150

14200

14250

14300

14350

14400

14450

14500

14550

14600

14650

14700

14750

14800

14850

14900

14950

15000

15050

15100

15150

15200

15250

15300

15350

15400

15450

15500

15550

15600

15650

15700

15750

15800

15850

15900

15950

16000

16050

16100

16150

16200

16250

16300

16350

16400

16450

16500

16550

16600

16650

16700

16750

16800

16850

16900

16950

17000

17050

17100

17150

17200

17250

17300

17350

17400

17450

17500

17550

17600

17650

17700

17750

17800

17850

17900

17950

18000

18050

18100

18150

18200

18250

18300

18350

18400

18450

18500

18550

18600

18650

18700

18750

18800

18850

18900

18950

19000

19050

19100

19150

19200

19250

19300

19350

19400

19450

19500

19550

19600

19650

19700

19750

19800

19850

19900

19950

20000

20050

20100

20150

20200

20250

20300

20350

20400

20450

20500

20550

20600

20650

20700

20750

20800

20850

20900

20950

21000

21050

21100

21150

21200

21250

21300

21350

21400

21450

21500

21550

21600

21650

21700

21750

21800

21850

21900

21950

22000

22050

22100

22150

22200

22250

22300

22350

22400

22450

22500

22550

22600

22650

22700

22750

22800

22850

22900

22950

23000

23050

23100

23150

23200

23250

23300

23350

23400

23450

23500

23550

23600

23650

23700

23750

23800

23850

23900

23950

24000

24050

24100

24150

24200

24250

24300

24350

24400

24450

24500

24550

24600

24650

24700

24750

24800

24850

24900

24950

25000

25050

25100

25150

25200

25250

25300

25350

25400

25450

25500

25550

25600

25650

25700

25750

25800

25850

25900

25950

26000

26050

26100

26150

26200

26250

26300

26350

26400

26450

26500

26550

26600

26650

26700

26750

26800

26850

26900

26950

27000

27050

27100

27150

27200

27250

27300

27350

27400

27450

27500

27550

27600

27650

27700

27750

27800

27850

27900

27950

28000

28050

28100

28150

28200

28250

28300

28350

28400

28450

28500

28550

28600

28650

28700

28750

28800

28850

28900

28950

29000

29050

29100

29150

29200

29250

29300

29350

29400

29450

29500

29550

29600

29650

29700

29750

29800

29850

29900

29950

30000

30050

30100

30150

30200

30250

30300

30350

30400

30450

30500

30550

30600

30650

30700

30750

30800

30850

30900

30950

31000

31050

31100

31150

31200

31250

31300

31350

31400

31450

31500

31550

31600

31650

31700

31750

31800

31850

31900

31950

32000

32050

32100

32150

32200

32250

32300

32350

32400

32450

32500

32550

32600

32650

32700

32750

32800

32850

32900

32950

33000

33050

33100

33150

33200

33250

33300

33350

33400

33450

33500

33550

33600

33650

33700

33750

33800

33850

33900

33950

34000

34050

34100

34150

34200

34250

34300

34350

34400

34450

34500

34550

34600

34650

34700

34750

34800

34850

34900

34950

35000

35050

35100

35150

35200

35250

35300

35350

35400

35450

35500

35550

35600

35650

35700

35750

35800

35850

35900

35950

36000

36050

36100

36150

36200

36250

36300

36350

36400

36450

36500

36550

36600

36650

36700

36750

36800

36850

36900

36950

37000

37050

37100

37150

37200

37250

37300

37350

37400

37450

37500

37550

37600

37650

37700

37750

37800

37850

37900

37950

38000

38050

38100

38150

38200

38250

38300

38350

38400

38450

38500

38550

38600

38650

38700

38750

38800

38850

38900

38950

39000

39050

39100

39150

39200

39250

39300

39350

39400

39450

39500

39550

39600

39650

39700

39750

39800

39850

39900

39950

40000

40050

40100

40150

40200

40250

40300

40350

40400

40450

40500

40550

40600

40650

40700

40750

40800

40850

40900

40950

41000

41050

41100

41150

41200

41250

41300

41350

41400

41450

41500

41550

41600

41650

41700

41750

41800

41850

41900

41950

42000

42050

42100

42150

42200

42250

42300

42350

42400

42450

42500

42550

42600

42650

42700

42750

42800

42850

42900

42950

43000

43050

43100

43150

43200

43250

43300

43350

43400

43450

43500

43550

43600

43650

43700

43750

43800

43850

43900

43950

44000

44050

44100

44150

44200

44250

44300

44350

44400

44450

44500

44550

44600

44650

44700

44750

44800

44850

44900

44950

45000

45050</

perchlorate. Positive and negative shoulder and toe speeds remain virtually unchanged. Similarly good results are obtained when 2,4-bis(4-ethylphenyl)-6-(4-styrylstyryl)pyrylium perchlorate is used.

### EXAMPLE III

Coating dopes are prepared in the manner described in example I using the materials set forth therein. The photoconductors employed are compounds 1-20 in Table I. In a darkened room, the surface of each of the photoconductive layers so prepared is charged to a potential of about +600 volts under a corona charger. The layer is then covered with a transparent sheet bearing a pattern of opaque and light-transmitting areas and exposed to the radiation from an incandescent lamp with an illumination intensity of about 75 meter-candles for 12 seconds. The resulting electrostatic latent image is developed in the usual manner by cascading over the surface of the layer a mixture of negatively charged black thermoplastic toner particles on glass beads functioning as carriers for the toner particles. A good reproduction of the pattern results in each instance. Similar results are obtained using a liquid developer.

The photoconducting compounds of this invention can generally be prepared by synthesis familiar to those skilled in the art. Typically, an intermediate Grignard or lithium derivative is prepared containing the desired substituents by conventional methods. The final product is prepared by reacting stoichiometric quantities of the intermediate with a Group IIIa metal halide or a Group IIIa metal halide containing the substituents desired in the final compound. A typical preparation is set forth below. Example IV describes the preparation of a typical tri-dialkylaminophenylborane wherein the alkyl moiety typically has 1 to 8 carbon atoms. The described procedure can be utilized to prepare the related organometallic compounds described above.

### EXAMPLE IV

A flask containing 17.2 g. (0.72 moles) of magnesium is heated at 100° C. for 1 hour, cooled to below 60° C. and treated with a 25 ml. portion of a solution of 55.2 g. (0.24 moles) of distilled p-bromo-N,N-diethylaniline in 240 ml. of dry tetrahydrofuran (distilled from calcium hydride). The reaction starts on heating under reflux. The remainder of the solution is added at such a rate as to maintain reflux. The resulting dark brown mixture is heated under reflux for 1 hour and then treated dropwise with a solution of 11.4 g. (0.08 moles) of boron trifluoride-ethyl ether in 100 ml. of dry tetrahydrofuran. The resulting mixture is heated under reflux for 2 hours. The solution is removed from unreacted magnesium and treated with ice and a dilute ammonium chloride solution. The solid which precipitates is dried in air at room temperature and purified by recrystallizing from boiling acetonitrile. The solid which results is dried in air at room temperature. 1.79 g. of white crystalline solid tri-p-diethylaminophenylborane having a melting point of 242°-273° C. are obtained.

Anal. Calc'd for  $C_{30}H_{42}N_3B$ : C, 79.1H, 9.2, B, 2.4; N, 9.2  
Found: C, 79.1; H, 9.1; B, 2.5; N, 9.3

The invention has been described in detail with particular reference to certain preferred embodiments thereof, but it will be understood that variations and modifications can be effected within the spirit and scope of the invention as described hereinabove and as defined in the appended claims.

I claim:

1. A photoconductive composition comprising an electrically insulating, polymeric binder having dispersed therein a photoconductor selected from the group consisting of a Group IIIa organometallic compound having at least one amino-aryl group attached to a Group IIIa metal atom.

2. The photoconductive composition as defined in claim 1 in which a sensitizer for said photoconductor is also present.

3. A photoconductive composition comprising a photoconductor which is a Group IIIa organometallic compound having attached to a Group IIIa metal atom (1) at least one amino-aryl group and (2) at least one substituent selected from the group consisting of a hydrogen atom, an alkyl group, an aryl group, a Group IIIa organometallic group, an alkoxy group, an aryloxy group and an amino group and a sensitizer for said photoconductor.

4. The photoconductive composition as defined in claim 3 wherein the Group IIIa organometallic compound is a borane.

5. The photoconductive composition as defined in claim 3 wherein the Group IIIa organometallic compound is a *p*-dialkylaminophenylborane.

6. The photoconductive composition as defined in claim 3 wherein the Group IIIa organometallic compound is *p*-diethylaminophenylborane.

7. The photoconductive composition as defined in claim 3 wherein the sensitizer is a pyrylium salt.

8. A photoconductive composition comprising a photoconductor represented by the formula:



wherein:

Ar is an arylene group;

D and E are each selected from the group consisting of an aryl group, an alkyl group, a hydrogen atom, an alkoxy group, an aryloxy group and an amino group;

M is a Group IIIa metal; and

R<sub>1</sub> and R<sub>2</sub> are each selected from the group consisting of an alkyl group, an aryl group and a hydrogen atom, and a sensitizer for said photoconductor.

9. The photoconductive composition as defined in claim 8 wherein M is boron.

10. The photoconductive composition as defined in claim 8 wherein R<sub>1</sub> and R<sub>2</sub> are each alkyl groups.

11. The photoconductive composition as defined in claim 8 wherein D and E are each *p*-dialkylaminophenyl groups.

12. The photoconductive composition as defined in claim 8 wherein Ar is a phenylene group.

13. The photoconductive composition as defined in claim 8 wherein the sensitizer is a pyrylium salt.

14. A photoconductive composition comprising a photoconductor represented by the formula:



wherein:

R<sub>1</sub> and R<sub>2</sub> are each selected from the group consisting of an alkyl group, an aryl group and hydrogen;

D and E are each selected from the group consisting of an aryl group, an alkyl group, hydrogen, an alkoxy group, an aryloxy group and an amino group;

M is a Group IIIa metal; and

X, T and Z are each selected from the group consisting of hydrogen, an alkyl group, an aryl group, an alkoxy group, an aryloxy group, a halogen atom and an amino group, and a sensitizer for said photoconductor.

15. The photoconductive composition as defined in claim 14 wherein M is boron.

16. The photoconductive composition as defined in claim 14 wherein D and E are each a *p*-dialkylaminophenyl group.

17. The photoconductive composition as defined in claim 14 wherein R<sub>1</sub> and R<sub>2</sub> are each an alkyl group.

18. The photoconductive composition as defined in claim 14 wherein the sensitizer is a pyrylium salt.

19. An electrophotographic element comprising a support having coated thereon a composition comprising a photoconductor which is a Group IIIa organometallic compound having at least one amino-aryl group attached to a Group IIIa metal atom.

20. An electrophotographic element comprising a support having coated thereon a composition comprising a photoconductor which is a Group IIIa organometallic compound having attached to a Group IIIa metal atom (1) at least one amino-aryl group and (2) at least one substituent selected from the group consisting of a hydrogen atom, an alkyl group, an aryl group, a Group IIIa organometallic group, an alkoxy group an aryloxy group and an amino group.

21. The electrophotographic element as defined in claim 20 wherein the Group IIIa organometallic compound is borane.

22. The electrophotographic element as defined in claim 20 wherein the Group IIIa organometallic compound is a *p*-dialkylaminophenylborane.

23. The electrophotographic element as defined in claim 20 wherein the Group IIIa organometallic compound is *p*-diethylaminophenylborane.

24. An electrophotographic element comprising a support having coated thereon a composition comprising a photoconductor represented by the formula:



wherein:

Ar is an arylene group;

D and E are each selected from the group consisting of an aryl group, an alkyl group, a hydrogen atom, an alkoxy group, an aryloxy group and an amino group;

M is a Group IIIa metal; and

R<sub>1</sub> and R<sub>2</sub> are each selected from the group consisting of an alkyl group, and aryl group and a hydrogen atom.

25. The electrophotographic element as defined in claim 24 wherein M is boron.

26. The electrophotographic element as defined in claim 24 wherein R<sub>1</sub> and R<sub>2</sub> are each an alkyl group.

27. The electrophotographic element as defined in claim 24 wherein D and E are each a *p*-dialkylaminophenyl group.

28. The electrophotographic element as defined in claim 24 wherein Ar is a phenylene group.

29. An electrophotographic element comprising a support having coated thereon a composition comprising a photoconductor represented by the formula:



wherein:

R<sub>1</sub> and R<sub>2</sub> are each selected from the group consisting of an alkyl group, an aryl group and hydrogen;

D and E are each selected from the group consisting of an aryl group, an alkyl group, hydrogen, an alkoxy group, an aryloxy group and an amino group;

M is a Group IIIa metal; and

25 X, T and Z are each selected from the group consisting of hydrogen, an alkyl group an aryl group, an alkoxy group, an aryloxy group, a halogen atom and an amino group.

30. The electrophotographic element as defined in claim 29 wherein M is boron.

31. The electrophotographic element as defined in claim 30 wherein D and E are each a *p*-dialkylaminophenyl group.

32. The electrophotographic element as defined in claim 30 wherein R<sub>1</sub> and R<sub>2</sub> are each an alkyl group.

33. An electrophotographic element comprising a support having coated thereon a photoconductive composition comprising 10 to about 60 weight percent of tri-*p*-diethylaminophenylborane as a photoconductor, 0.005 to about 5.0 weight percent of [4-(*p*-diethylaminophenyl)-2,6-diphenylthiapyrylium perchlorate] as a sensitizer and a polymeric binder for said photoconductor.